

Patented Dec. 26, 1922.

1,439,939

# UNITED STATES PATENT OFFICE.

JUD M. BLAKE, OF CHICAGO HEIGHTS, ILLINOIS, ASSIGNOR TO AMERICAN MANGANESE STEEL COMPANY, OF CHICAGO, ILLINOIS, A CORPORATION OF MAINE.

## LOW-PERCENTAGE MANGANESE STEEL.

No Drawing.

Application filed July 9, 1919. Serial No. 309,567.

*To all whom it may concern:*

Be it known that I, JUD M. BLAKE, a citizen of the United States, residing at Chicago Heights, in the county of Cook and 5 State of Illinois, have invented new and useful Low-Percentage Manganese Steel, of which the following is a specification.

An object of the present invention is to produce a steel which will have a degree of 10 hardness that will adapt it to resist erosion or wear, with a low coefficient of flowing action.

Commercial manganese steel usually containing from 10 to 14% manganese has been 15 found to be unsuccessful for many commercial purposes, owing to the flowing action of the steel under the influence of the forces which it encounters in use, for instance, pan bottoms, roll tires, and scrapers employed in 20 the wet grinding of clay in the manufacture of fire bricks.

I have found by experiment that a very satisfactory steel can be produced for the foregoing purposes, as well as other uses 25 where similar forces are encountered, by adding to a good commercial grade of steel produced by the open hearth, Bessemer, or electric furnace processes, a very much smaller percentage of manganese than is employed in 30 ordinary commercial manganese steel. I prefer to employ for this purpose from 3.50 to 4.50% of manganese. I have found in practice that good results are obtained by using 4.25% of manganese in a steel containing about .42% of carbon and .25% of silicon. The analysis of phosphorus in the 35 steel tested was .07% while its sulphur content was .03%. These constituents, however, aggregating about .10% which I regard as 40 impurities and as not bearing upon the result obtained.

In producing the steel, the manganese content is added to the heat after the steel is otherwise developed by any improved known 45 process, and the heat is then poured to produce the commercial articles desired. After pouring, the cooling of the castings is preferably controlled in order to regulate the degree of hardness obtained. For instance, 50 the castings may be placed in a suitable annealing furnace and subjected to heat treatment of from 1325° to 1375° F., the furnace being held at this temperature until the heat 55 has thoroughly penetrated the entire section of the casting, after which the furnace is

shut off and the casting allowed to cool with the furnace. For certain classes of work it is desirable to permit castings to cool quickly and in other classes of work to cool slowly. Low manganese steel castings made in accordance with this invention may be cooled 60 quickly by removing the castings from the furnace after the same have been subjected to heat treatment for cooling in the air and may be cooled slowly by permitting the castings to remain in the heat treatment furnace so that the temperature of the castings will fall with that of the furnace. The hardness thus obtained will be suitable for many commercial purposes. 70

If, however, a greater hardness is required, and particularly if a high degree of toughness is not needed in the commercial purpose for which the casting is intended, the cooling may be permitted to proceed more rapidly, 75 as by cooling the castings in the open air, or in a furnace without applied heat or with a modified application of heat.

I claim:

1. A commercial steel containing manganese and carbon in the proportions of about 4.25% manganese and .42% of carbon. 80

2. The herein-described process of producing articles of low percentage manganese steel, which consists in adding, to a suitable bath of molten steel, manganese in the proportion of not over 4.50%, pouring the steel to produce the castings, subjecting the castings to heat treatment in an annealing furnace at 1325° F. to 1375° F. until the heat 90 has fully penetrated the entire section of the castings, and then allowing the castings to cool in the atmosphère. 95

3. The herein-described process of producing articles of low percentage manganese steel, which consists in adding, to a suitable bath of molten steel, manganese in the proportion of not over 4.50%, pouring the steel to produce the castings, subjecting the castings to heat treatment in an annealing furnace at 1325° to 1375° F. until the heat has 100 fully penetrated the entire section of the castings, and then allowing the castings to cool in the furnace. 105

4. Annealed cast steel containing about 4.25% of manganese, about .42% of carbon and about .25% of silicon.

Signed at Chicago Heights, Illinois, this third day of July, 1919.

JUD M. BLAKE.